

March 24, 1959

L. C. KRCHMA

2,878,650

METHOD OF COOLING THERMOPLASTIC AND VISCOUS MATERIALS

Filed June 10, 1955



INVENTOR

LUDWIG C. KRCHMA  
BY  
*Raymond Lubell*  
ATTORNEY

1

2,878,650

**METHOD OF COOLING THERMOPLASTIC AND VISCOUS MATERIALS**

Ludwig C. Krchma, Kansas City, Mo., assignor to Socony Mobil Oil Company, Inc., a corporation of New York

Application June 10, 1955, Serial No. 514,414

3 Claims. (Cl. 62—98)

The cooling of thermoplastic materials, of which highly viscous oils, and particularly high melting point asphalts, are typical, presents a rather serious problem. This invention is directed to an improved method therefor. It will be discussed with specific reference to highly viscous oils.

Cooling of highly viscous oils through higher temperature ranges, say down to about 400° F. from the processing temperatures at which they are produced, usually of the order of 400° F. to 800° F. and above, is normally not too serious a problem, and is capable of being handled in the usual exchangers, and the like.

Below about 400° F., the problem becomes different. The oil being cooled becomes increasingly viscous, and proper contact of the material with the tube walls of a tubular heat exchanger becomes difficult to obtain because of lack of turbulence in the oil stream. Pumping pressures become increasingly costly because of increasing viscosity, particularly when it is realized that poor contact of oil and tube wall require greatly increased length of oil passage due to decrease of heat transfer through tube walls. It is at the same time rather impractical to pass the cooling fluid through the tubes of a conventional exchanger while passing the oil around the tubes because of fouling and coking difficulties often arising from the very nature of the heavy oils when so handled.

In many instances, it is desirable both to store these materials at elevated temperatures, say of the order of 300° F. to 400° F., but to pass them therefrom to a processing step, such as mixing, or the like which must be conducted at a lower temperature, such as a temperature of from 225 to 275° F.

Obviously, it is not economical to attempt to cool such products by mere storage. (It is quite common to ship hot asphalt in tank cars for quite long distances without substantial cooling.)

It is therefore an object of this invention to provide a method of cooling heavy, viscous oils, such as high melting point asphalts, and the like, without the use of heat transfer through surfaces separating the oil from the coolant. It is a further object to provide a rapid and effective method for such cooling, one readily susceptible to accurate control. It is an object to provide a non-hazardous method for cooling, and one that employs a minimum of costly equipment.

This invention is based upon the discovery that, quite contrary to expectation, cooling can be readily effected by admixing liquid water with a confined moving stream of hot viscous oil that is immiscible with water.

This is quite contrary to previous experience within the oil industry, for it is well known that the adventitious mixture of water with hot viscous oil results in the formation of foam and froth in volumes many, many times greater than that of the oil and water involved. Major care is always taken when pumping heavy oil, above the boiling point of water, into a storage tank, to see that the storage tank is substantially free of acci-

2

dentially present water. Even in applying asphalt saturants to roofing felts, papers, and the like, the small amounts of moisture present in the felts, etc., from storage in ordinary atmospheres, frequently gives very serious foaming troubles.

This method is also quite different from the older method, well known in the asphalt blowing art, of controlling the temperature of a blowing still by introducing water, or propane, etc. (i.e., a material vaporizable below the temperature of the still content), into the oil being blown. It has been appreciated for some time that water, when introduced into an agitated body of hot oil, evaporates therefrom without much foaming difficulty. The blowing air in the blowing still provides such agitation. The present method contemplates admixing the water with hot oil, an operation which, in the light of prior experience, could be expected to be conducive to excessive foam production.

This method also differs from proposals for cooling asphalt blowing stills by spraying water into the space above the air-agitated oil in such a still. There, the water contacts only the surface of the oil body. Here, the water is intimately mixed with hot oil.

In order that this invention may be more readily understood, reference is now made to the drawing which forms a part of this specification.

In this drawing, the single figure of which is highly diagrammatic in form, 1 represents a tank containing hot, high melting point asphalt, which is to be cooled. This oil is pumped through pipe 2 by pump 3 over through pipe 4 into tank 5. Both tanks 1, and 5, are rather conventional in form, and equipped, as shown, with the usual roof hatches 6, and may be equipped, if desired, with air aspirators such as 7, actuated by steam or air from valved pipe 8. Such tanks, in comparatively small sizes, around 1000 bbls. or less, are commonly used in specification asphalt manufacture. At point 9, a controlled small amount of liquid water is introduced from pipe 10, under pressure of pump 11. This water may be withdrawn from tank 12, or from water main 13, 14. The amount of water so injected may be controlled in any of several ways. Pump 11 may be a metering pump such as those commonly used for injection of chemicals etc., into a flowing fluid stream. Control may be effected by valve 15, in a usual manner, in which case, if pump 11 be a positive displacement type, a pressure controlled bypass 16, around pump 11 will be required. Or an automatic setup, indicated in very general form by observation point 17 and responsive valve 18, can be used, the observation at 17 being rate of flow, temperature, or a combination of these. All such methods of control and proportioning of two streams of liquid from mere manual control to elaborate proportioning instrumentation, are well known in the art. In general, for heavier, viscous oils, the simpler the control, the better. In most cases, with a pump 3 capable of operating at reasonably constant discharge, manual control at valve 15 will be adequate.

It will also be realized that the hot oil to pump 3 may come from some other source, such as from a manufacturing operation through pipe 19, or that the contents of tank 5 may be recirculated to cooling, as by pipe 20, or that any combination of such sources could be used.

The proportioning of water to oil is dependent upon the rate of cooling desired, and the major criterion of control is that substantially no liquid water shall be discharged from the end of the mixing pipe into the tank. Even this is advisable rather than mandatory, for a small amount of free water can be tolerated, particularly when the tank oil is well above the boiling point of water.

Contrary to expectation, the amount of water so added

can range up to that necessary to effect substantial cooling in a single pass. For example, an asphalt of 225° F. soft point can be cooled in a single pass from about 380° to about 320° F., requiring about 4.8 gallons of 62° F. water per minute, pumped into oil flowing at a rate of about 265 barrels per hour. If desired, the operation can be conducted at lower rates.

The piping sizes are in no way critical, except that the diameter and length of the mixing pipe, and the nature of the water injection fitting should be such as to secure adequate mixing before discharge. Since such devices are quite common in the oil and other industries for various purposes and the manner of calculating sizes, etc., is well known in the art, no discussion is offered here.

Actual operating results of a series of cooling runs are set forth below in Table I.

4  
material to a temperature above its soft point and above the boiling point of water; discharging the resulting mixture into a vaporizing space, and permitting the separation and escape of water vapor.

5  
5. The method of cooling highly viscous heated petroleum oil fractions, of the nature of asphaltic residues and the like, which comprises: passing the oil which is at a temperature substantially above the boiling point of water, through a conduit as a confined stream; continuously admixing liquid water in controlled small quantities with said material while passing through said conduit, to cool said material to a temperature above its soft point and above the boiling point of water; discharging the resulting mixture into a vaporizing space; and permitting the separation and escape of water vapor.

10  
15  
3. The method of cooling highly viscous heated petro-

Table I

| Trial Runs | Asphalt Soft Point | Asphalt Temp. Before Inject., degrees | Asphalt Temp. After Inject., degrees | Total Quant. Asphalt Barrels | Asphalt Transfer Rate, Bbls./Hr. | Water Temp., degrees | Highest Water Rate, Gals./Min. | Ave. Water Rate, Gals./Min. | Total Water Quant., Gallons | Time Of Inject. In Hrs. | B.t.u.'s/Hr. Removed From Asphalt | Total B.t.u.'s Removed From Asphalt |
|------------|--------------------|---------------------------------------|--------------------------------------|------------------------------|----------------------------------|----------------------|--------------------------------|-----------------------------|-----------------------------|-------------------------|-----------------------------------|-------------------------------------|
| 1          | 220                | 350                                   | 332                                  | 288                          |                                  | 60                   | 2.5                            | 1.43                        | 86                          | 1.00                    | 798,000                           | 798,000                             |
| 2          | 220                | 332                                   | 313                                  | 288                          |                                  | 60                   | 3.0                            | 1.73                        | 78                          | 0.75                    | 967,000                           | 725,000                             |
| 3          | 225                | 340                                   | 325                                  | 350                          |                                  | 60                   | 3.0                            | 1.75                        | 105                         | 1.00                    | 975,000                           | 975,000                             |
| 4          | 225                | 337                                   | 297                                  | 350                          |                                  | 50                   | 3.5                            | 2.10                        | 218                         | 1.75                    | 1,167,000                         | 2,040,000                           |
| 5          | 231                | 350                                   | 288                                  | 280                          | 140                              | 60                   | 3.5                            | 3.00                        | 360                         | 2.00                    | 1,670,000                         | 3,340,000                           |
| 6          | 224                | 360                                   | 290                                  | 280                          |                                  | 65                   | 5.5                            | 3.90                        | 350                         | 1.50                    | 2,150,000                         | 3,225,000                           |
| 7          | 226                | 435                                   | 285                                  | 250                          |                                  | 60                   | 6.5                            | 4.60                        | 689                         | 2.50                    | 2,596,000                         | 6,490,000                           |
| 8          | 225                | 380                                   | 320                                  | 200                          | 265                              | 62                   | 5.0                            | 4.80                        | 220                         | 0.75                    | 2,706,000                         | 2,030,000                           |
| 9          | 225                | 320                                   | 300                                  | 260                          |                                  | 62                   | 6.0                            | 5.50                        | 110                         | 0.33                    | 3,054,000                         | 1,018,000                           |

15 and 8—One pass operation.

In the above runs, runs 5 and 8 are once-through runs. All others are recirculating runs, in which the oil to be cooled was withdrawn from the same tanks into which the mixed oil and water streams discharged.

In all of these runs, the water flashed to steam and readily disengaged from the asphalt. Asphalt and foam samples taken from the tanks immediately after cooling showed substantially no moisture. Foam was not voluminous. There was no serious hazard apparent from foam, from fire, or from explosion. The process is simple and economical, from the standpoint of operating and from equipment and maintenance considerations.

I claim:

1. The method of cooling a thermoplastic material which is not miscible with water, which comprises: passing the thermoplastic material which is at a temperature substantially above the boiling point of water, through a conduit as a confined stream; continuously admixing liquid water in controlled small quantities with said material while passing through said conduit, to cool said

leum oil fractions, of the nature of asphaltic residues and the like, which comprises: passing the oil which is at a temperature of about 400° F., through a conduit as a confined stream; continuously admixing liquid water, in an amount from about 0.5 to about 4 percent by volume of the oil, with said oil while passing through said conduit, to cool said oil to a temperature above its soft point and above the boiling point of water; discharging the resulting mixture into a vaporizing space; and permitting the separation and escape of water vapor.

45  
References Cited in the file of this patent

UNITED STATES PATENTS

|           |                    |                |
|-----------|--------------------|----------------|
| 1,135,506 | Dubbs              | Apr. 13, 1915  |
| 1,587,111 | Fogler             | June 1, 1926   |
| 2,062,374 | Noel               | Dec. 1, 1936   |
| 2,231,544 | McCorqudale et al. | Feb. 11, 1941  |
| 2,265,801 | Cooke              | Dec. 9, 1941   |
| 2,421,968 | Schutte            | June 10, 1947  |
| 2,652,594 | Campbell           | Sept. 22, 1953 |